

May 4, 1965

L. M. BROWNING ET AL

3,182,012

CATALYTIC HYDROCRACKING

Filed Sept. 12, 1958

2 Sheets-Sheet 1



III fig. 1



III fig. 2



III fig. 3



III fig. 4

INVENTORS

Lewis M. Browning  
BY Carl W. Street

Raymond W. Barclay  
ATTORNEY

May 4, 1965

L. M. BROWNING ET AL

3,182,012

CATALYTIC HYDROCRACKING

Filed Sept. 12, 1958

2 Sheets-Sheet 2



Fig. 5



Fig. 6



Fig. 7

INVENTORS  
Lewis M. Browning  
BY Carl W. Street  
Raymond W. Barclay  
ATTORNEY

3,182,012

## CATALYTIC HYDROCRACKING

Lewis M. Browning, Needham, Mass., and Carl W. Streed, Sewell, N.J., assignors to Socony Mobil Oil Company, Inc., a corporation of New York

Filed Sept. 12, 1958, Ser. No. 760,646

8 Claims. (Cl. 208—111)

This invention relates to an improved hydrocarbon conversion catalyst characterized by a predominant proportion of alumina and specified minor proportions of molybdena, silica, and cobalt oxide combined in a particular manner. The invention is further directed to a process wherein a high boiling hydrocarbon or hydrocarbon mixture, for example, a petroleum fraction, is subjected to cracking in the presence of hydrogen and the aforementioned catalyst.

As is well known, cracking refers generally to operations wherein a long chain hydrocarbon or a mixture of high molecular weight hydrocarbons is converted into a shorter chain hydrocarbon or into a mixture of lower molecular weight hydrocarbons. Cracking accomplished solely as a result of the high operational temperature employed is known as thermal cracking while cracking effected in the presence of catalyst is ordinarily known as catalytic cracking. Cracking carried out in the presence of hydrogen is referred to as hydrocracking.

Catalytic cracking of petroleum hydrocarbons has heretofore been carried out at temperatures in the range of 800° F. to 1100° F. Such high temperatures have been 30 inefficient from an economics standpoint and undesirable from an operational standpoint, resulting in the production of unwanted coke, relatively large amounts of dry gas, and excess quantities of C<sub>4</sub> hydrocarbons. The production of coke and dry gas represents a loss, thereby 35 bringing about an overall decrease in the yield of useful cracked product.

As is well known, charge stocks heretofore employed in catalytic cracking operations have been selected petroleum stocks. Thus, heavy residual stocks, as well as cycle 40 stocks obtained from the catalytic cracking of non-refractory petroleum cracking stocks, have not been suitable for catalytic cracking processes because of their inherent coke-forming characteristics and the excessive amounts of dry gas produced. Accordingly, the supply of available crack- 45 ing stocks has been somewhat restricted.

Cracking operations carried out in the presence of hydrogen at relatively high temperatures and under high pressure, i.e. hydrocracking, do not impose the aforesaid 50 limitations on the type of utilizable charge stock. Thus, cycle stocks, heavy residuals, etc. can be cracked in hydrocracking operations. Conventional operations of this type, however, have many disadvantages. Thus, in order to maintain catalyst activity at a desired level and to avoid a heavy deposition of coke on the catalyst, it has 55 been necessary to employ excessively high hydrogen pressures of the order of at least about 3500 pounds per square inch and preferably much higher.

There is accordingly, at the present time, great interest 60 in the petroleum industry in developing a moderate pressure hydrocracking process. This interest arises from the ability of hydrocracking to substantially increase both the quantity and quality of naphtha and fuel oil that a petroleum refinery can produce from crude oil. These advantages have been amply demonstrated by the aforementioned high-pressure hydrocracking operations. The high 65 cost of high-pressure hydrocracking, necessitating the use of expensive high-pressure equipment, has prevented its wide spread use, hence the interest in developing a less expensive, moderate-pressure process which will retain 70 many of the demonstrated advantages, but at acceptable cost.

In accordance with the present invention, it has been discovered that cracking of hydrocarbons in the presence of hydrogen and a particular catalyst permits the use of appreciably lower reaction temperatures and pressures. Thus, it has been found that cracking of hydrocarbons can be effected in the presence of hydrogen and in the presence of a catalyst consisting essentially of alumina, silica and the oxides of molybdenum and cobalt combined in such manner that the resulting composite is characterized by a silica content of about 15 to about 40 percent by weight, a molybdenum trioxide content of about 3 to about 20 percent by weight, a cobalt oxide content of about 1 to about 8 percent by weight and the remainder alumina. Preferably the catalyst has a composition of about 15 to about 25 weight percent silica, about 7 to about 16 weight percent molybdenum trioxide, about 2 and about 4.5 percent cobalt oxide and the remainder alumina. Such catalyst employed in the process of the invention has been found to afford a highly favorable distribution of products of high quality. The process described herein has the further advantage of being applicable for catalytically hydrocracking a wide variety of charge stocks, including heavy residual and refractory charge stocks.

The present invention provides a process for cracking hydrocarbons and particularly petroleum hydrocarbon fractions having an initial boiling point of at least about 400° F., a 50 percent point of at least about 500° F. and an end boiling point of at least 600° F. and boiling substantially continuously between said initial boiling point and said end boiling point by contacting said fractions with the above catalyst in the presence of hydrogen at a hydrogen partial pressure between about 700 and about 3000 pounds per square inch gauge at a liquid hourly space velocity of between about 0.1 and about 10 at a temperature between about 600° F. and about 950° F., employing a molar ratio of hydrogen to hydrocarbon charge between about 2 and about 80.

We are aware that it has heretofore been proposed to desulfurize hydrocarbon fractions in the presence of certain catalytic composites containing alumina, silica, cobalt oxide and molybdena. The hydrocracking process described herein is distinguishable from such desulfurizing processes. Thus, there are at least four differences between the cracking process of this invention and the aforesaid desulfurizing operations. First of all, it may be noted that the processes are carried out for two different purposes. Cracking is used to convert high boiling hydrocarbon fractions into low boiling hydrocarbon fractions, while desulfurizing is carried out for the sole purpose of removing sulfur from the charge stock undergoing treatment. Secondly, the silica content of the above type catalysts useful in desulfurization is substantially lower than the silica content of the catalysts employed in the present hydrocracking process. A third difference relates to the chemical reactions involved in the processes. In desulfurizing, it is desired to remove sulfur from a hydrocarbon by reaction of the sulfur compounds with hydrogen with resulting formation of H<sub>2</sub>S. Cracking, on the other hand, involves conversion of high boiling hydrocarbons to lower boiling hydrocarbons by selective breakage of carbon to carbon bonds. A still further distinction resides in the fact that the hydrocracking process of this invention is generally carried out at pressures outside the range specified for desulfurization. It will accordingly be appreciated that the aforementioned desulfurizing processes utilizing catalysts containing alumina, silica, molybdena and cobalt oxide are distinct from the hydrocracking process of this invention.

Catalysts proposed for hydrocracking operations have, heretofore, consisted almost entirely, of active hydrogenating components dispersed on an existing active cracking

base such as platinum on silica-alumina, molybdena on silica-alumina or of supported metal oxides or sulfides that have, to varying degrees, both hydrogenating and cracking activity such as nickel sulfide on alumina, tungsten disulfide on clay and the like. Neither of the above type catalysts has proven satisfactory for moderate pressure hydrocracking. When tested these catalysts have shown a lack in one or more of the following: the ability to retain activity during use; a good balance between cracking and hydrogenating activities; or the recovery of activity when carbonaceous deposits are removed after a period of use.

Following the teachings of this invention, it has been found that highly effective catalysts for use in moderate pressure hydrocracking can be obtained by intimately compositing the oxides of aluminum, cobalt, molybdenum and silicon in particularly specified proportion. The catalysts of this invention have been found to be capable of affording unexpected performance in hydrocracking petroleum fractions at moderate pressures, i.e. generally not in excess of a hydrogen partial pressure of about 3000 pounds per square inch.

The catalyst components of silica, alumina, cobalt oxide and molybdenum trioxide may be combined in any suitable manner. It has been discovered, however, as will be evident from data set forth hereinbelow, that it is preferable to produce the catalyst by mechanical admixture of the silica and alumina-containing components, rather than by chemical compositing of these oxides such as, for example, by cogelation. Either the silica or alumina-containing component may prior to admixture with the other have deposited thereon one or both of the other catalyst components, i.e. cobalt oxide and/or molybdenum trioxide. Thus, the catalyst of the invention may be produced by mechanically admixing silica with alumina which has previously been impregnated with the oxides of molybdenum and cobalt. Alternatively, the catalyst may result from mechanical admixture of alumina with silica which has previously been impregnated with the oxides of molybdenum and cobalt. Another method of combining the catalyst components involves admixture of silica impregnated with either molybdenum trioxide or cobalt oxide with alumina impregnated with the other of such metal oxides. It is also feasible, and in some aspects preferable, to initially intimately admix the silica and alumina components and thereafter to impregnate the resulting silica-alumina composite with the oxides of molybdenum and cobalt. The composite obtained, in accordance with any of the above techniques, is dried and calcined to obtain the finished catalyst.

While the alumina component is the predominating constituent of the present catalyst and has, of itself, no hydrocracking activity, its careful preparation is essential to the production of the catalyst affording the desired activity in the contemplated conversion of the hydrocarbon charge. The alumina when properly prepared exerts a synergistic effect with the other catalyst components.

The alumina component of the present catalyst is a porous alumina not adversely affected by the temperature conditions of the instant process, having a surface area greater than 100 square meters per gram and which may extend up to 500 square meters per gram or more. Catalysts prepared from alumina having a surface area of 100 square meters per gram or less have a considerably higher aging rate when employed in the instant low pressure hydrocracking process in comparison to catalysts in which the alumina component initially is characterized by a surface area in substantial excess of 100 square meters per gram. The term "surface area" as used herein designates the surface area as determined by the adsorption of nitrogen according to the method of Brunauer et al. Journal American Chemical Society 60, 309 et seq. (1938). As noted above, the alumina itself, is devoid of or exerts negligible catalytic activity under the reaction conditions at which the present hydrocracking process is

carried out. The density of the alumina employed, i.e. the bulk density thereof, will usually be within the range of .2 to 2.0 grams/cc. and more particularly between about 0.4 and about 1.2 grams/cc.

- 5 The alumina component of the present catalyst may be prepared by commingling a suitable basic compound including ammonium hydroxide, ammonium carbonate, etc. with an acidic compound of aluminum including the chloride, bromide, iodide, fluoride, sulfate, phosphate, nitrate, acetate, etc. or by the addition of a suitable acidic compound including hydrogen chloride, sulphuric acid, phosphoric acid, etc. to an alkaline compound of the metal as for example, an alkali metal aluminate such as sodium aluminate. The resultant aluminum hydroxide 10 is usually washed to remove soluble impurities and then is dried at a temperature of from 200° F. to about 600° F. for a period of from 1 to 24 hours or more. In one method the dried alumina is formed into particles of definite size and shape in any suitable manner such as 15 casting, pelleting, extruding, etc. and then is subjected to calcination at a temperature of from about 600° to about 1600° F. In another embodiment the alumina may be formed into particles of spherical shape by dropping a suitable alumina sol into a suitable medium which may 20 comprise air, an inert atmosphere, as for example nitrogen, carbon monoxide, etc. or into an oil or other suitable immiscible liquid. The resultant spheroids are then washed, dried and calcined in the manner hereinbefore set forth. Alternatively, the alumina may be prepared 25 in the form of a precipitate by controlled reaction of aluminum metal with water in the presence of a mercury compound whereby the aluminum undergoes amalgamation and the resulting amalgamated aluminum reacts with the water to form alumina.
- 30 The silica component is initially prepared in the form of a hydrogel or gelatinous precipitate. Preferably, the silica component is prepared in the form of a hydrogel by reaction between sodium silicate and an acid, such as sulfuric acid, while maintaining the pH of the reaction mixture generally below about 6 and preferably in the approximate range of 3.5 to 5. The initially formed hydrosol of silica undergoes gelation after lapse of a suitable period of time to silica hydrogel. The time of gelation can be controlled within desired limits by well known means such as adjustment in the temperature 35 or solids concentration of the reaction mixture or hydrosol produced therefrom. The resulting hydrogel is thereafter water-washed, base-exchanged to remove zeolitic sodium and dried. If it is desired to prepare silica initially free of alkali metal ions, such may be accomplished by effecting hydrolysis of alkyl silicates, i.e. ethyl silicate. The silica hydrogel may be produced in the 40 form of granules or in the form of a mass, which is thereafter broken up into pieces or particles of desired size. Alternatively, the silica hydrogel may be produced 45 in the form of spheroidal bead particles by methods such as those described by Marisic in U.S. 2,384,946, or in the form of uniformly shaped particles prepared by casting or extrusion methods. It is also feasible to initially produce silica in the form of finely divided 50 particles of requisite particle size by employing techniques used in the preparation of fluid catalyst particles, for example, by spraying or rapid agitation of a hydrosol to form minute particles of hydrosol that set to particles of hydrogel, which, upon drying yield discrete particles 55 of silica gel. Generally, it is preferred that the silica component before admixture with the alumina-containing component be in a finely divided state, generally of a particle size finer than 50 mesh (Tyler) and preferably of a particle size within the approximate range of 60 to 200 mesh (Tyler). The above indicated finely divided 60 state of silica can be obtained either during initial formation of the silica or by grinding larger size pieces to the requisite particle size.
- 65 The alumina and silica, prepared as above, may be

composed by mechanical admixture and thereafter impregnated with cobalt oxide and molybdenum trioxide; or either of these components, prior to admixture with the other, may be impregnated with suitable compounds of molybdenum and cobalt to effect deposition thereon of cobalt oxide and molybdenum trioxide. The base material, i.e., alumina, silica, or composite resulting from admixture of silica and alumina is contacted with an impregnating solution of a cobalt compound, such as cobalt nitrate, and of a molybdenum compound, such as ammonium molybdate. In one method, the particles of base material are initially subjected to a vacuum to remove air from the pores thereof and while maintaining the vacuum, the above-described impregnating solution is brought into contact with the particles of base material. Alternatively, the base material, for example, in the form of an aqueous slurry may be impregnated with the solution of molybdenum compound and cobalt compound. It is understood that any other suitable method of commingling particles of the base material with the impregnating solution may be employed.

In another embodiment, separate impregnating solutions of the molybdenum compound and of the cobalt compound are prepared and are composited successively with the base material either with or without intervening heating of the support. In general, using this technique, it is preferred to composite the molybdenum component first and then the cobalt component, although the reverse procedure may be employed. After the impregnation, the base material is dried and then calcined to convert the metal compounds to the oxides.

Other suitable cobalt compounds for effecting deposition of cobalt oxide on the base material may be employed including, for example, cobalt ammonium nitrate, cobalt ammonium chloride, cobalt ammonium sulfate, cobalt bromide, cobalt bromate, cobalt chloride, cobalt chlorate, cobalt fluoride and cobalt fluorate. In similar manner, other suitable compounds of molybdenum may be employed. Suitable soluble molybdenum compounds include molybdenum tetrabromide, molybdenum oxydibromide, molybdenum tetrachloride, molybdenum oxydichloride, molybdenum oxypentachloride and molybdenum oxytetrafluoride.

The silica-containing component preferably in finely divided form is intimately mixed with the alumina-containing component which likewise is in a finely divided state preferably having a particle size within the approximate range of 60 to 200 mesh (Tyler). After thorough mixing of the components, the resulting mixture is formed by pelleting, casting, molding or other means into pieces of desired size and shape such as rods, spheres, pellets, etc. After forming into particles of desired size, the resulting particles are dried and thereafter calcined at an elevated temperature in the approximate range of 600 to 1200° F. It is understood that either the silica and alumina-containing components may prior to admixture be impregnated with molybdenum trioxide and cobalt oxide or that the mixed composite of silica and alumina may subsequently be impregnated with the oxides of molybdenum and cobalt.

The impregnating solution ordinarily contains the cobalt and molybdenum compounds in the proportions desired in the final catalyst and the impregnation is controlled to produce a final catalyst containing these components in the desired concentrations. The concentrations of the cobalt and molybdenum oxides in the catalyst described herein may respectively range from about 1 to about 8 percent by weight and from about 3 to about 20 percent by weight of the final catalyst. The preferred catalysts contain cobalt oxide (CoO) in a concentration of from about 2.0 to about 4.5 percent and molybdenum trioxide (MoO<sub>3</sub>) in a concentration of from about 7 to 16 percent by weight of the final catalyst. After impregnation the final composite generally is dried at a temperature of from about 200° to about 600° F. for a

period of from about 2 to 24 hours or more and thereafter calcined at a temperature of from about 600° to 1200° F. for a period of from about 1 to 12 hours or more.

It is an essential feature of the catalyst of this invention that the silica content thereof be at least about 15 percent by weight. Composites containing amounts of silica less than about 15 percent by weight do not possess the requisite hydrocracking activity observed in the case of the present catalyst. The cobalt oxide content of the catalyst, as noted hereinabove, is preferably between about 2 and about 4.5 percent by weight. A higher cobalt oxide content increased the saturation of the fuel oil and cycle stock, but decreased the combined naphtha and fuel oil yield and caused a slight increase in the aging rate of the catalyst. An increase in the molybdenum trioxide content of the catalyst was found to raise the heavy naphtha to fuel oil ratio and to increase the saturation of the fuel oil and cycle stock.

The catalyst described herein desirably has a surface area within the approximate range of 200 to 370 square meters per gram. Composites having surface areas of less than about 200 square meters per gram were found to have considerably higher aging rates in the present low pressure hydrocracking process and accordingly are less preferred than catalysts characterized by surface areas within the aforementioned range. Within this range, the hydrocracking activity of the catalyst was observed to increase with increasing surface area.

The process of this invention may be carried out in any suitable equipment for catalytic operations. The process may be operated batchwise. It is preferable, however, and generally more feasible to operate continuously. Accordingly, the process is adapted to operations using a fixed bed of catalyst. Also, the process can be operated using a moving bed of catalyst wherein the hydrocarbon flow may be concurrent or countercurrent to the catalyst flow. A fluid type of operation wherein the catalyst is carried in suspension in the hydrocarbon charge may feasibly be employed using the present catalyst.

Hydrocracking, in accordance with the present process, is generally carried out at a temperature between about 600° F. and about 950° F. and preferably between about 700° F. and about 900° F. The hydrogen partial pressure in such operation is generally within the range of about 700 and about 3000 pounds per square inch gauge and preferably about 1000 and 2000 pounds per square inch gauge. The liquid hourly space velocity of fresh feed i.e. the liquid volume of hydrocarbons per hour per volume of catalyst is between about 0.1 and about 10 and preferably between about 0.25 and about 4. In general, the molar ratio of hydrogen to hydrocarbon charge employed, i.e. fresh feed, is between about 2 and about 80 and preferably between about 5 and about 40.

Hydrocarbon charge stocks undergoing cracking in accordance with this invention comprise hydrocarbons, mixtures of hydrocarbons, and particularly hydrocarbon fractions having an initial boiling point of at least about 400° F., a 50 percent point of at least 500° F. and an end boiling point of at least 600° F. and boiling substantially continuously between said initial boiling point and end boiling point. Such hydrocarbon fractions include gas oils, residual stocks, cycle stocks, whole topped crudes and heavy hydrocarbon fractions obtained by the destructive hydrogenation of coal, tars, pitches, asphalts and the like. As will be recognized, the distillation of higher boiling petroleum fractions (about 750° F.) must be carried out under vacuum in order to avoid thermal cracking. The boiling temperatures utilized herein, however, are expressed for convenience in terms of the boiling point corrected to atmospheric pressure.

The term "gas oil" as employed in the art includes a variety of petroleum stocks. As utilized herein, this term, unless further modified, includes any fraction dis-

tilled from petroleum which has an initial boiling point of at least about 400° F., a 50 percent point of at least about 500° F. and an end boiling point of at least about 600° F. and boiling substantially continuously between the initial boiling point and the end boiling point. The exact boiling range of a gas oil accordingly will be determined by the initial boiling point, the 50 percent point, and by the end boiling point. In practice, petroleum distillations have been effected under vacuum at temperatures as high as 1200° F. (corrected to atmospheric pressure). Accordingly, in the broad sense, a gas oil is a petroleum fraction which boils substantially continuously within an approximate range of 400° F. to 1200° F., the 50 percent point being at least about 500° F. Thus, a gas oil may boil over the entire approximate range of 400° F. to 1200° F. or over an intermediate range such as 500° F. to 900° F.

A residual stock is any fraction which is not distilled. Accordingly, any fraction, regardless of its initial boiling point, which includes heavy bottoms, such as tars, asphalts, etc., is a residual fraction. A residual stock may be the portion of the crude remaining undistilled at about 1200° F. or it may be made up of a gas oil fraction plus the portion undistilled at about 1200° F.

A whole topped crude is the entire portion of the crude remaining after the light ends; i.e., the portion boiling up to about 400° F. has been removed by distillation. Accordingly, such a fraction includes the entire gas oil fraction and the undistilled portion of the crude petroleum boiling above about 1200° F. If desired, the residual fractions and the whole topped crude may be deasphalted by any suitable well-known means. Such deasphalting treatment, however, is not considered necessary for charge stocks utilizable in the process of this invention.

The refractory cycle stocks are cuts of cracked stocks which boil above the gasoline boiling range usually between about 400° F. and about 850° F. The refractory cycle stocks can be charged to the process of this invention, together with a fresh petroleum charge stock or the refractory cycle stocks may be charged to the process alone.

The hydrocracking selectivities of the catalysts described herein are evaluated by comparing their product distributions at fixed conversion levels. The conversion is defined as 100 minus the volume percent of charge remaining in the 650° F.+ boiling range. The products considered are dry gas (C<sub>1</sub>-C<sub>3</sub>), C<sub>4</sub> material, light naphtha (C<sub>5</sub>-180° F.), heavy naphtha (180-390° F.), fuel oil (390-650° F.) and cycle stock (650° F.+). An overall measure of selectivity is the total yield of C<sub>5</sub>-650° F. material at any conversion level, since this range contains the more valuable products.

The hydrocracking activity of a catalyst, as this term is utilized herein, is defined as the temperature required to achieve a given conversion level.

The catalyst aging rate, as this term is utilized herein, is defined as the rate of temperature increase (°F./day) required to maintain constant conversion with all operating conditions except temperature held constant.

The following examples will serve to illustrate the process of this invention without limiting the same:

#### EXAMPLE 1

A composite of cobalt and molybdenum oxides on alumina in the form of  $\frac{1}{8}$ " x  $\frac{1}{8}$ " pellets and prepared by impregnation of alumina gel with approximately 3 percent by weight CoO and approximately 9.5 percent by weight MoO<sub>3</sub>, was crushed to a particle size of less than 100 mesh (Tyler). Approximately 85 parts by weight of the crushed material were mixed with approximately 43 parts by weight of silica hydrogel, containing about 35 weight percent SiO<sub>2</sub> and 65 weight percent water, and having a particle size of less than 60 mesh (Tyler). The resulting composite was intimately

mixed by ball-milling the components for about 24 hours, at which time the particles were of 14 to 15 microns average size. The ball-milled material was then pelleted to  $\frac{1}{16}$ " diameter by  $\frac{1}{16}$ " thick pellets. The pellets, so obtained, were then tempered for 3 hours at 1000° F. in dry air. The resulting product contained, on a weight basis, about 2.5 percent CoO, about 8 percent MoO<sub>3</sub>, about 15 percent SiO<sub>2</sub> and about 74.5 percent Al<sub>2</sub>O<sub>3</sub> and possessed a surface area of approximately 220 square meters per gram.

#### EXAMPLE 2

A catalyst was prepared following the procedure of Example 1 but by mixing approximately 95 parts by weight of the crushed component of cobalt and molybdenum oxides on alumina with approximately 14 parts by weight of the crushed silica hydrogel. The resulting product contained, on a weight basis, about 3 percent CoO, about 9 percent MoO<sub>3</sub>, about 5 percent SiO<sub>2</sub> and about 83 percent Al<sub>2</sub>O<sub>3</sub> and possessed a surface area of approximately 188 square meters per gram.

#### EXAMPLE 3

A catalyst was prepared following the procedure of Example 1 but by mixing approximately 75 parts by weight of the crushed component of cobalt and molybdenum oxides on alumina with approximately 72 parts by weight of the crushed silica hydrogel. The resulting product contained, on a weight basis, about 2 percent CoO, about 7 percent MoO<sub>3</sub>, about 25 percent SiO<sub>2</sub> and about 66 percent Al<sub>2</sub>O<sub>3</sub> and was characterized by a surface area of approximately 263 square meters per gram.

#### EXAMPLE 4

This example is not illustrative of the invention but is included for purposes of comparison. In this example, no silica was combined with the composite of cobalt and molybdenum oxides on alumina but this material was ground, repelleted, and tempered under the conditions of Example 1. The resulting product contained, on a weight basis, about 3 percent CoO, about 9.5 percent MoO<sub>3</sub>, and about 87.5 percent Al<sub>2</sub>O<sub>3</sub> and had a surface area of approximately 185 square meters per gram.

Properties of the above four catalysts are shown in Table I below:

Table I

| Example                            | 4     | 2     | 1     | 3     |
|------------------------------------|-------|-------|-------|-------|
| Catalyst composition, wt. percent: |       |       |       |       |
| CoO                                | 3     | 3     | 2.5   | 2     |
| MoO <sub>3</sub>                   | 9.5   | 9     | 8     | 7     |
| Al <sub>2</sub> O <sub>3</sub>     | 87.5  | 83    | 74.5  | 66    |
| SiO <sub>2</sub>                   | 0     | 5     | 15    | 25    |
| Density, g./cc.:                   |       |       |       |       |
| Packed                             | 0.92  | 1.10  | 1.03  | 0.89  |
| Particle                           | 1.55  | 1.71  | 1.62  | 1.45  |
| Real                               | 3.72  | 3.54  | 3.38  | 3.16  |
| Surface area, m. <sup>2</sup> /g.  | 185   | 188   | 220   | 263   |
| Pore volume, cc./g.                | 0.373 | 0.301 | 0.320 | 0.374 |
| Pore diameter, Å                   | 81    | 64    | 58    | 57    |

It will be seen from the above table that an effect of increasing silica addition is to increase the surface area and to decrease the average pore diameter of the resulting catalyst.

The above catalysts of Examples 1-4 were tested in hydrocracking a charge of a 650 to 920° F. boiling range Guico gas oil. Hydrocracking was carried out under a set of standard operating conditions, which have been found by experience to afford satisfactory evaluation of catalyst performance, thereby permitting a direct comparison of each of the catalysts to be made. The standard conditions involved conversion of the gas oil charge at 0.5 liquid hourly space velocity and at 1500 pounds per square inch pressure, utilizing a hydrogen to hydrocarbon charge mol ratio of about 40 corresponding to 14,500 standard cubic feet of hydrogen per barrel of charge. Hydrogen and the charge stock were mixed together at the above pressure, heated to reaction temperature and

passed downward through a bed of the catalyst contained in a test unit. Hot effluent from the bottom of the catalyst bed was cooled and separated at the pressure utilized in the unit into gas and liquid product streams. The liquid product stream was stabilized at atmospheric pressure before being sampled for distillation and analysis. The gases recovered from the high pressure separation and from stabilizing the liquid product were sampled and analyzed. Activity of the catalysts was evaluated by operating the catalyst bed at three temperature levels selected so as to cover 40 to 95 volume percent conversion of the gas oil charge to material boiling below 650° F.

Performance of the control catalyst containing no silica, i.e. the catalyst of Example 4, in converting the gas oil charge under the standard test conditions is shown at three conversion levels of 40, 70 and 95 volume percent in Table II below:

Table II

| Conversion (100%, yield of 650° F.+ liquid), vol. percent | 40    | 70    | 95    | 20 |
|-----------------------------------------------------------|-------|-------|-------|----|
| Reactor temperature, ° F.                                 | 776   | 820   | 862   |    |
| Product yield, based on charge:                           |       |       |       |    |
| Dry gas, wt. percent                                      | 2.0   | 3.5   | 7.5   | 25 |
| Total C <sub>4</sub> 's, vol. percent                     | 1.0   | 2.0   | 6.0   |    |
| C <sub>5</sub> 's, light naphtha, vol. percent            | 2.5   | 5.0   | 10.5  |    |
| Heavy naphtha, vol. percent                               | 5.5   | 17.0  | 37.0  |    |
| Fuel oil, vol. percent                                    | 33.0  | 51.0  | 50.0  |    |
| Cycle stock, vol. percent                                 | 60.0  | 30.0  | 5.0   |    |
| Total liquid recovery, vol. percent                       | 102.0 | 105.0 | 108.5 | 30 |
| Hydrogen consumption, s.c.f./b.                           |       | 750   | 1,050 |    |
| Performance inspections:                                  |       |       |       |    |
| Propane in dry gas, wt. percent                           | 45    | 45    |       |    |
| Heavy naphtha/fuel oil volume ratio                       | 0.17  | 0.33  | 0.74  |    |
| Isomerization (weight ratio):                             |       |       |       |    |
| i/n C <sub>4</sub> 's                                     | 0.4   | 0.4   | 35    |    |
| i/n C <sub>5</sub> 's                                     | 0.5   | 0.5   |       |    |
| Product inspections:                                      |       |       |       |    |
| Heavy naphtha:                                            |       |       |       |    |
| Paraffins, vol. percent                                   | 37    | 43    |       |    |
| Naphthenes, vol. percent                                  | 42    | 36    |       |    |
| Aromatics, vol. percent                                   | 21    | 21    |       |    |
| Olefins, vol. percent                                     | 0     | 0     |       |    |
| Fuel oil:                                                 |       |       |       |    |
| Diesel index                                              | 42    | 51    |       |    |
| Aromatics, vol. percent                                   | 38    | 32    |       |    |
| Olefins, vol. percent                                     | 9     | 3     |       |    |

Performance of the catalyst containing 5 weight percent silica, i.e. the catalyst of Example 2, in converting the gas oil charge under the standard test conditions is shown at three conversion levels of 40, 70 and 95 volume percent in Table III below:

Table III

| Conversion (100%, yield of 650° F.+ liquid), vol. percent | 40    | 70    | 95    | 50    |
|-----------------------------------------------------------|-------|-------|-------|-------|
| Reactor temperature, ° F.                                 | 777   | 811   | 848   |       |
| Product yield, based on charge:                           |       |       |       |       |
| Dry gas, wt. percent                                      | 2.0   | 3.5   | 6.0   |       |
| Total C <sub>4</sub> 's, vol. percent                     | 1.5   | 3.5   | 7.5   |       |
| C <sub>5</sub> 's, light naphtha, vol. percent            | 1.5   | 5.5   | 13.0  |       |
| Heavy naphtha, vol. percent                               | 7.5   | 23.0  | 46.0  |       |
| Fuel oil, vol. percent                                    | 32.5  | 45.0  | 39.0  |       |
| Cycle stock, vol. percent                                 | 60.0  | 30.0  | 5.0   | 60    |
| Total liquid recovery, vol. percent                       | 103.0 | 107.0 | 110.5 |       |
| Hydrogen consumption, s.c.f./b.                           |       | 440   | 800   | 1,150 |
| Performance inspections:                                  |       |       |       |       |
| Propane in dry gas, wt. percent                           | 35    | 45    | 45    |       |
| Heavy naphtha/fuel oil volume ratio                       | 0.23  | 0.51  | 1.18  |       |
| Isomerization (weight ratio):                             |       |       |       |       |
| i/n C <sub>4</sub> 's                                     | 1.3   | 1.0   |       |       |
| i/n C <sub>5</sub> 's                                     | 2.4   | 2.0   |       |       |
| Product inspections:                                      |       |       |       |       |
| Heavy naphtha:                                            |       |       |       |       |
| Paraffins, vol. percent                                   | 31    | 37    | 44    |       |
| Naphthenes, vol. percent                                  | 50    | 46    | 38    |       |
| Aromatics, vol. percent                                   | 18    | 17    | 18    |       |
| Olefins, vol. percent                                     | 1     | 0     | 0     |       |
| Fuel oil:                                                 |       |       |       |       |
| Diesel index                                              | 43    | 49    | 53    |       |
| Aromatics, vol. percent                                   | 26    | 26    | 28    |       |
| Olefins, vol. percent                                     | 15    | 9     | 3     |       |
| Cycle stock: Diesel index                                 | 76    | 84    | 79    |       |

Performance of the catalyst containing 15 weight percent silica, i.e. the catalyst of Example 1, in converting the gas oil charge under the standard test conditions is shown at three conversion levels of 40, 70 and 95 volume percent in Table IV below:

Table IV

| Conversion (100%, yield of 650° F.+ liquid), vol. percent | 40    | 70    | 95    |
|-----------------------------------------------------------|-------|-------|-------|
| Reactor temperature, ° F.                                 | 757   | 787   | 815   |
| Product yield, based on charge:                           |       |       |       |
| Dry gas, wt. percent                                      | 1.5   | 3.0   | 5.0   |
| Total C <sub>4</sub> 's, vol. percent                     | 1.5   | 4.5   | 9.0   |
| C <sub>5</sub> 's, light naphtha, vol. percent            | 2.0   | 6.5   | 15.5  |
| Heavy naphtha, vol. percent                               | 9.0   | 26.5  | 48.5  |
| Fuel oil, vol. percent                                    | 32.0  | 41.0  | 36.0  |
| Cycle stock, vol. percent                                 | 60.0  | 30.0  | 5.0   |
| Total liquid recovery, vol. percent                       | 104.5 | 108.5 | 114.0 |
| Hydrogen consumption, s.c.f./b.                           | 560   | 860   | 1,270 |
| Performance inspections:                                  |       |       |       |
| Propane in dry gas, wt. percent                           | 60    | 65    | 65    |
| Heavy naphtha/fuel oil volume ratio                       | 0.28  | 0.66  | 1.35  |
| Isomerization (weight ratio):                             |       |       |       |
| i/n C <sub>4</sub> 's                                     | 1.4   | 1.1   |       |
| i/n C <sub>5</sub> 's                                     | 2.5   | 2.1   |       |
| Product inspections:                                      |       |       |       |
| Heavy naphtha:                                            |       |       |       |
| Paraffins, vol. percent                                   | 29    | 33    | 49    |
| Naphthenes, vol. percent                                  | 52    | 48    | 39    |
| Aromatics, vol. percent                                   | 18    | 14    | 12    |
| Olefins, vol. percent                                     | 1     | 0     | 0     |
| Fuel oil:                                                 |       |       |       |
| Diesel index                                              | 44    | 53    | 63    |
| Aromatics, vol. percent                                   | 28    | 24    | 20    |
| Olefins, vol. percent                                     | 15    | 10    | 6     |
| Cycle stock: Diesel index                                 | 73    | 86    | 88    |

Performance of the catalyst containing 25 weight percent silica, i.e. the catalyst of Example 3, in converting the gas oil charge under the standard test conditions is shown at three conversion levels of 40, 70 and 95 volume percent in Table V below:

Table V

| Conversion (100%, yield of 650° F.+ liquid), vol. percent | 40    | 70    | 95    |
|-----------------------------------------------------------|-------|-------|-------|
| Reactor temperature, ° F.                                 | 756   | 788   | 810   |
| Product yield, based on charge:                           |       |       |       |
| Dry gas, wt. percent                                      | 1.5   | 3.0   | 4.0   |
| Total C <sub>4</sub> 's, vol. percent                     | 1.0   | 5.0   | 10.0  |
| C <sub>5</sub> 's, light naphtha, vol. percent            | 2.0   | 6.5   | 16.0  |
| Heavy naphtha, vol. percent                               | 8.5   | 26.0  | 47.5  |
| Fuel oil, vol. percent                                    | 32.5  | 41.0  | 36.0  |
| Cycle stock, vol. percent                                 | 60.0  | 30.0  | 5.0   |
| Total liquid recovery, vol. percent                       | 104.0 | 108.5 | 114.5 |
| Hydrogen consumption, s.c.f./b.                           | 450   | 810   | 1,240 |
| Performance inspections:                                  |       |       |       |
| Propane in dry gas, wt. percent                           | 60    | 65    | 65    |
| Heavy naphtha/fuel oil volume ratio                       | 0.26  | 0.63  | 1.32  |
| Isomerization (weight ratio):                             |       |       |       |
| i/n C <sub>4</sub> 's                                     | 1.4   | 1.1   |       |
| i/n C <sub>5</sub> 's                                     | 2.5   | 2.1   |       |
| Product inspections:                                      |       |       |       |
| Heavy naphtha, vol. percent:                              |       |       |       |
| Paraffins                                                 | 27    | 37    | 48    |
| Naphthenes                                                | 51    | 48    | 38    |
| Aromatics                                                 | 21    | 15    | 14    |
| Olefins                                                   | 1     | 0     | 0     |
| Fuel oil:                                                 |       |       |       |
| Diesel index                                              | 48    | 54    | 60    |
| Aromatics, vol. percent                                   | 27    | 24    | 23    |
| Olefins, vol. percent                                     | 12    | 8     | 6     |
| Cycle stock: Diesel index                                 | 74    | 83    | 80    |

Graphical comparisons of the above four catalysts are set forth in the attached drawing wherein:

FIGURE 1 shows the relationship between reactor temperature and catalyst silica content.

FIGURE 2 shows the relationship between the dry gas yield and catalyst silica content.

FIGURE 3 shows the relationship between the yield of total C<sub>4</sub>'s and catalyst silica content.

FIGURE 4 shows the relationship between the yield of C<sub>5</sub>'s-light naphtha and catalyst silica content.

FIGURE 5 shows the relationship between the yield of heavy naphtha and catalyst silica content.

FIGURE 6 shows the relationship between the yield of fuel oil and catalyst silica content.

FIGURE 7 shows the relationship between diesel index of the fuel oil product (390-650° F. boiling range) and catalyst silica content.

It will be seen from reference to FIGURE 1 that the catalysts of 15 and higher weight percent silica content were much more active than catalysts having a silica content of less than about 15 weight percent. Activities are compared here in terms of the catalyst bed temperature required to convert the charge oil. Thus, it will be seen that the average catalyst bed temperature required to obtain 40, 70 and 95 percent conversions of the gas oil charge decreased steadily with increasing silica content of the catalyst until a silica content of about 15 weight percent was reached. Thereafter, the required temperature leveled off with increasing silica content in the catalyst. Low catalyst bed temperatures, as will be realized, are highly desirable in commercial hydrocracking operations both from a process and mechanical design standpoint.

It will be seen from the data of Tables II to V, as well as from FIGS. 2 to 6, that the catalysts of 15 and greater weight percent silica gave greatly superior product distributions than are obtainable with the catalyst of no silica or with the catalyst containing only 5 weight percent silica. Thus, FIGURES 2 to 6 show the product distributions obtained at 40, 70 and 95 percent conversions of the gas oil plotted against the silica content of the catalysts. The yield of total C<sub>4</sub>'s, C<sub>5</sub>'s-light naphtha, and heavy naphtha increase as the silica content of the catalyst increased from 0 to about 15 weight percent and thereafter level off with further increases in the silica content of the catalyst. The dry gas yield decreases substantially with increasing silica content from 0 to 15 weight percent at the 95 percent conversion level. The fuel oil yield decreases as the silica content of the catalyst increases from 0 to 15 weight percent and thereafter levels off with an increasing content of silica.

It will be noted by reference to FIG. 7 where the diesel index of the 390-650° F. boiling range product fuel oil is plotted against the silica content of the catalyst that the diesel index increased with increasing silica content until the catalyst contained about 15 weight percent and thereafter leveled off with increasing content of silica.

The following examples illustrate various methods for preparing the catalyst of the invention including comparative evaluation of the catalyst products so obtained:

#### EXAMPLE 5

A catalyst using the procedure of Example 1 was prepared. The resulting product contained, on a weight basis, 2.9 percent CoO, 8 percent MoO<sub>3</sub>, 15.2 percent SiO<sub>2</sub> and 73.9 percent Al<sub>2</sub>O<sub>3</sub> and was characterized by a surface area of approximately 238 square meters per gram.

#### EXAMPLE 6

Alumina and silica hydrogel, containing about 35 weight percent SiO<sub>2</sub> and 65 weight percent water, were dried separately for 16 hours at 240° F. and were then crushed to a particle size of less than 60 mesh (Tyler). A composite containing about 82 parts by weight of alumina and about 18 parts by weight of silica, on a dry basis, was formed by mixing these crushed materials. The resulting composite was ball-milled dry for about 24 hours, at which time the particles were of 14 to 15 microns average size. The ball-milled material was then pelleted to 1/8" diameter by 1/16" thick pellets. The pellets, so obtained, were then calcined for 3 hours at 900° F. in dry air.

The pellets of silica and alumina were then pretreated with carbon dioxide and impregnated under vacuum with sufficient ammonium molybdate solution to yield a composite containing about 10 weight percent MoO<sub>3</sub> on a dry basis. The impregnated pellets were dried for 8 hours at 240° F. in

hours at 240° F. and calcined for 3 hours at 900° F. in dry air.

5 The pellets were again pretreated with carbon dioxide and impregnated under vacuum with sufficient cobaltous nitrate solution to yield a composite containing about 3 weight percent CoO on a dry basis. The impregnated pellets were then dried for 8 hours at 240° F. and calcined for 3 hours at 900° F. in dry air, yielding the finished catalyst.

#### EXAMPLE 7

10 A cogel containing, on a dry basis, 79 weight percent of alumina and 21 weight percent of silica was prepared by mixing 1000 cc. of a sodium silicate solution containing 1.4 weight percent Na<sub>2</sub>O, 4.5 weight percent SiO<sub>2</sub> and 94.1 weight percent water with 1000 cc. of 30.6 weight percent aqueous sodium aluminate solution in the presence of 800 cc. of a 34.2 weight percent aqueous solution of citric acid. The resulting cogel was aged for about 16 hours at room temperature and was then base-exchanged with 20 weight percent aqueous ammonium sulfate solution. The cogel was then washed with water until sulfate free. The washed cogel was dried for 24 hours at 240° F. to 250° F. in 100 percent steam and then ball-milled dry for 16 hours. The dried cogel was pelleted into 1/8" diameter by 1/16" thick pellets.

15 The resulting pellets were pretreated with carbon dioxide and impregnated under vacuum with sufficient ammonium molybdate solution to yield a composite containing about 7.6 weight percent MoO<sub>3</sub> on a dry basis. The impregnated pellets were dried for 8 hours at 240° F. and calcined for 3 hours at 900° F. in dry air.

20 The pellets were again pretreated with carbon dioxide and impregnated under vacuum with sufficient cobaltous nitrate solution to yield a composite containing about 3 weight percent CoO on a dry basis. The impregnated pellets were then dried for 8 hours at 240° F. and calcined for 3 hours at 900° F. in dry air, yielding the finished catalyst.

#### EXAMPLE 8

25 Alumina was extruded into 1/8" diameter particles. The extruded particles were dried at 230° F. and calcined for 3 hours at 1000° F. in dry air. The calcined particles were pretreated with carbon dioxide and impregnated under vacuum with a solution containing ammonium molybdate and cobaltous nitrate in amounts sufficient to yield a composite containing about 10 weight percent MoO<sub>3</sub> and about 3 weight percent CoO, on a dry basis. The alumina particles were soaked for about 16 hours in the impregnating solution. The impregnated alumina was then dried at 230° F. and calcined for 3 hours at 1000° F. in dry air.

30 The impregnated alumina was crushed to a particle size of less than 60 mesh (Tyler) and mixed with silica hydrogel, containing about 35 weight percent SiO<sub>2</sub> and about 65 weight percent water, having a particle size of less than 60 mesh (Tyler), in such proportions that the mixture contained about 85 weight percent impregnated alumina and about 15 weight percent silica, on a dry basis. The resulting composite was intimately mixed by dry ball-milling for about 24 hours, at which time the particles were of 14 to 15 microns average size. The ball-milled material was then pelleted to 1/8" diameter, by 1/16" thick pellets. The pellets, so obtained, were then tempered for 3 hours at 1000° F. in dry air.

#### EXAMPLE 9

35 Alumina was mixed with water to form a slurry containing about 9 cc. of water per gram of dry alumina. Aqueous solutions of ammonium molybdate and cobaltous nitrate were added to this slurry in amounts sufficient to yield a composite containing about 12 weight percent MoO<sub>3</sub> and 3 weight percent CoO, on a dry basis. The resulting composite was aged for 16 hours at room temperature.

Silica hydrogel, containing about 35 weight percent  $\text{SiO}_2$  and 65 weight percent water, and having a particle size of less than 60 mesh (Tyler), was added to the alumina-molybdena-cobalt oxide slurry in an amount sufficient to yield a composite containing 15 weight percent  $\text{SiO}_2$  on a dry basis. The resulting composite was intimately mixed by wet ball-milling for about 24 hours,

It will be seen from the above comparative data that the catalysts of Examples 6 and 8, despite the difference in their methods of preparation, have similar hydrocracking performance.

Comparative evaluation of the catalysts of Examples 5 and 7 at 30, 50 and 70 volume percent conversion level shown in Table VII below:

Table VII

| Conversion (100%, yield of 650° F. liquid) vol. percent | 30        |           | 50        |           | 70        |           |
|---------------------------------------------------------|-----------|-----------|-----------|-----------|-----------|-----------|
|                                                         | Example 7 | Example 5 | Example 7 | Example 5 | Example 7 | Example 5 |
| Reactor temperature, ° F.                               | 750       | 710       | 790       | 760       | 805       | 795       |
| Product yield, based on charge:                         |           |           |           |           |           |           |
| Dry gas, wt. percent                                    | 1.0       | 1.0       | 2.0       | 1.5       | 6.0       | 2.5       |
| Total $\text{C}_4$ 's, vol. percent                     | 0.5       | 1.0       | 1.5       | 1.5       | 3.5       | 3.5       |
| $\text{C}_5$ , light naphtha, vol. percent              | 1.5       | 0.5       | 3.5       | 2.5       | 5.0       | 6.5       |
| Heavy naphtha, vol. percent                             | 8.0       | 5.0       | 17.0      | 15.5      | 23.0      | 30.0      |
| Fuel oil, vol. percent                                  | 24.0      | 26.5      | 34.0      | 38.0      | 44.5      | 41.0      |
| Cycle stock, vol. percent                               | 70.0      | 70.0      | 50.0      | 50.0      | 30.0      | 30.0      |
| Total liquid recovery, vol. percent                     | 104.0     | 103.0     | 106.0     | 107.5     | 106.0     | 111.0     |
| $\text{C}_5$ , fuel oil yield, vol. percent             | 33.5      | 32.0      | 54.5      | 56.0      | 72.5      | 77.5      |
| Hydrogen consumption, s.c.f./b.                         | 750       | 750       | 1,100     | 1,100     | 1,450     | 1,450     |
| Product inspections:                                    |           |           |           |           |           |           |
| Heavy naphtha:                                          |           |           |           |           |           |           |
| Paraffins, vol. percent                                 | 22        | 16        | 27        | 21        | 32        | 28        |
| Olefins, vol. percent                                   | 3         | 3         | 0         | 2         | 0         | 1         |
| Naphthenes, vol. percent                                | 45        | 56        | 50        | 56        | 48        | 56        |
| Aromatics, vol. percent                                 | 30        | 25        | 23        | 21        | 20        | 15        |
| Fuel oil: Diesel index                                  | 31        | 35        | 40        | 47        | 50        | 59        |

after which time the particles were of about 14 to 15 microns average size. The ball-milled material was then dried at 230° F., pelleted to  $\frac{1}{8}$ " diameter by  $\frac{1}{16}$ " thick pellets and calcined for 3 hours at 1000° F. dry air.

The above catalysts were tested in hydrocracking a charge of a 650 to 800° F. boiling range West Texas gas oil. The test conditions involved conversion of the gas oil charge at 1 liquid hourly space velocity and at 2000 pounds per square inch pressure, utilizing a hydrogen to hydrocarbon mol ratio of about 40, corresponding to 14,500 standard cubic feet of hydrogen per barrel of charge. Activity of the catalysts was evaluated by operating the catalyst bed at varying temperature levels selected so as to cover 30 to 70 volume percent conversion of the gas oil charge to material boiling below 650° F.

Comparative evaluation of the catalysts of Examples 6 and 8 at a 50 and 70 volume percent conversion level is shown in Table VI below:

Table VI

| Conversion (100%, yield of 650° F. liquid), vol. percent | 50        |           | 70        |           |
|----------------------------------------------------------|-----------|-----------|-----------|-----------|
|                                                          | Example 8 | Example 6 | Example 8 | Example 6 |
| Reactor temperature, ° F.                                | 790       | 775       | 822       | 810       |
| Product yield, based on charge:                          |           |           |           |           |
| Dry gas, wt. percent                                     | 2.0       | 1.5       | 3.0       | 2.5       |
| Total $\text{C}_4$ 's, vol. percent                      | 1.5       | 1.5       | 3.5       | 3.0       |
| $\text{C}_5$ , light naphtha, vol. percent               | 3.5       | 3.0       | 8.0       | 6.5       |
| Heavy naphtha, vol. percent                              | 18.0      | 16.5      | 33.0      | 29.5      |
| Fuel oil, vol. percent                                   | 34.0      | 35.5      | 36.0      | 40.5      |
| Cycle stock, vol. percent                                | 50.0      | 50.0      | 30.0      | 30.0      |
| Total liquid recovery, vol. percent                      | 107.0     | 106.5     | 110.5     | 109.5     |
| $\text{C}_5$ , fuel oil yield, vol. percent              | 55.5      | 55.0      | 77.0      | 76.5      |
| Hydrogen consumption, s.c.f./b.                          | 1,000     | 900       | 1,300     | 1,200     |
| Product inspections:                                     |           |           |           |           |
| Heavy naphtha:                                           |           |           |           |           |
| Paraffins, vol. percent                                  | 25        | 26        | 33        | 34        |
| Olefins, vol. percent                                    | 1         | 5         | 2         | 5         |
| Naphthenes, vol. percent                                 | 54        | 46        | 51        | 44        |
| Aromatics, vol. percent                                  | 20        | 23        | 14        | 17        |
| Fuel oil:                                                |           |           |           |           |
| Diesel index                                             | 43        | 43        | 56        | 52        |
| Saturates, vol. percent                                  | 64        | 55        | 70        | 66        |
| Olefins, vol. percent                                    | 8         | 22        | 5         | 14        |
| Aromatics, vol. percent                                  | 28        | 23        | 25        | 20        |

It will be seen from the above comparative data that the catalyst of Example 7 wherein the preparation method involved impregnation of cogelled silica-alumina with cobalt and molybdenum oxides was less active, particularly at the lower conversions, than the catalyst of Example 5 prepared by mechanical addition of silica to a composite of alumina previously impregnated with the oxides of cobalt and molybdenum. At the higher conversions, the product distribution employing the catalyst of Example 7 is inferior to that obtained with the catalyst of Example 5. Thus with the catalyst of Example 7, the dry gas make is higher and the naphtha and total product yields are lower than those obtained with the catalyst of Example 5. In addition, the hydrogenating activity of the Example 7 catalyst is lower than that of the Example 5 catalyst, as shown by the lower diesel indices of the fuel oil. It will accordingly be appreciated that in view of the foregoing, it is preferred to employ a catalyst wherein the alumina-containing and silica-containing components are composited by mechanical admixture thereof rather than by cogelation.

However, it is to be understood that the above description is merely illustrative of preferred embodiments of the invention, of which many variations may be made within the scope of the following claims by those skilled in the art without departing from the spirit thereof.

We claim:

1. A process for cracking hydrocarbon fractions which comprises contacting, in the presence of hydrogen, a hydrocarbon fraction having an initial boiling point of at least about 400° F., a 50 percent point of at least about 500° F. and an end point of at least about 600° F. and boiling substantially continuously between said initial boiling point and said end point with a catalyst consisting essentially of 15 to 40 percent by weight silica, 1 to 8 percent cobalt oxide, 3 to 20 percent by weight molybdenum trioxide and remainder alumina prepared by impregnating the alumina component with the cobalt oxide and molybdenum trioxide components, mechanically mixing the resulting impregnated product with the silica component, drying and calcining the resulting composite at an elevated temperature, said contacting being effected at a temperature between about 600° F. and about 950° F., a liquid hourly space velocity between about 0.1 and

about 10, a hydrogen partial pressure between about 700 and about 3000 pounds per square inch gauge employing a molar ratio of hydrogen to hydrocarbon charge between about 2 and about 80.

2. A process for cracking hydrocarbon fractions which comprises contacting, in the presence of hydrogen, a hydrocarbon fraction having an initial boiling point of at least about 400° F., a 50 percent point of at least about 500° F. and an end point of at least about 600° F. and boiling substantially continuously between said initial boiling point and said end point with a catalyst consisting essentially of 15 to 40 percent by weight silica, 1 to 8 percent by weight cobalt oxide, 3 to 20 percent by weight molybdenum trioxide and remainder alumina prepared by mechanically mixing the alumina and silica components and impregnating the resulting composite with the cobalt oxide and molybdenum trioxide components, drying and calcining the resulting product at an elevated temperature, said contacting being effected at a temperature between about 600° F. and about 950° F., a liquid hourly space velocity between about 0.1 and about 10, a hydrogen partial pressure between about 700 and about 3000 pounds per square inch gauge employing a molar ratio of hydrogen to hydrocarbon charge between about 2 and about 80.

3. A process for cracking hydrocarbon fractions which comprises contacting, in the presence of hydrogen, a hydrocarbon fraction having an initial boiling point of at least about 400° F., a 50 percent point of at least about 500° F. and an end point of at least about 600° F. and boiling substantially continuously between said initial boiling point and said end point with a catalyst characterized by a surface area in the approximate range of 200 to 370 square meters per gram and consisting essentially of 15 to 40 percent by weight of silica, 1 to 8 percent by weight cobalt oxide, 3 to 20 percent by weight molybdenum trioxide and remainder alumina prepared by intimately mixing silica hydrogel with alumina having a surface area greater than 100 square meters per gram, impregnating the resulting composite with the cobalt oxide and molybdenum oxide components, drying and calcining the resulting product at an elevated temperature, said contacting being effected at a temperature between about 600° F. and about 950° F., a liquid hourly space velocity between about 0.1 and about 10, a hydrogen partial pressure between about 700 and about 3000 pounds per square inch gauge employing a molar ratio of hydrogen to hydrocarbon charge between about 2 and about 80.

4. A process for cracking hydrocarbon fractions which comprises contacting, in the presence of hydrogen, a hydrocarbon fraction having an initial boiling point of at least about 400° F., a 50 percent point of at least about 500° F. and an end point of at least about 600° F. and boiling substantially continuously between said initial boiling point and said end point with a catalyst characterized by a surface area within the approximate range of 200 to 370 square meters per gram consisting essentially of 15 to 40 percent by weight silica, 1 to 8 percent by weight cobalt oxide, 3 to 20 percent by weight molybdenum trioxide and remainder alumina prepared by impregnating alumina having a surface area greater than 100 square meters per gram with the cobalt oxide and molybdenum trioxide components, mechanically mixing the resulting impregnated product with silica hydrogel, drying and calcining the resulting composite at an ele-

vated temperature, said contacting being effected at a temperature between about 600° F. and about 950° F., a liquid hourly space velocity between about 0.1 and about 10, a hydrogen partial pressure between about 700 and about 3000 pounds per square inch gauge employing a molar ratio of hydrogen to hydrocarbon charge between about 2 and about 80.

5. A catalyst, characterized by hydrocracking activity, and consisting essentially of 15 to 40 percent by weight silica, 1 to 8 percent cobalt oxide, 3 to 20 percent by weight molybdenum trioxide and remainder alumina prepared by impregnating the alumina component with the cobalt oxide and molybdenum trioxide components, mechanically mixing the resulting impregnated product with the silica component, drying and calcining the resulting composite at an elevated temperature.

6. A catalyst, characterized by hydrocracking activity and consisting essentially of 15 to 40 percent by weight silica, 1 to 8 percent by weight cobalt oxide, 3 to 20 percent by weight molybdenum trioxide and remainder alumina prepared by mechanically mixing the alumina and silica components and impregnating the resulting composite with the cobalt oxide and molybdenum trioxide components, drying and calcining the resulting product at an elevated temperature.

7. A catalyst characterized by a surface area in the approximate range of 200 to 370 square meters per gram and consisting essentially of 15 to 40 percent by weight of silica, 1 to 8 percent by weight cobalt oxide, 3 to 20 percent by weight molybdenum trioxide and remainder alumina prepared by intimately mixing silica hydrogel with alumina having a surface area greater than 100 square meters per gram, impregnating the resulting composite with the cobalt oxide and molybdenum oxide components, drying and calcining the resulting product at an elevated temperature.

8. A catalyst characterized by a surface area within the approximate range of 200 to 370 square meters per gram consisting essentially of 15 to 40 percent by weight silica, 1 to 8 percent by weight cobalt oxide, 3 to 20 percent by weight molybdenum trioxide and remainder alumina prepared by impregnating alumina having a surface area greater than 100 square meters per gram with the cobalt oxide and molybdenum trioxide components, mechanically mixing the resulting impregnated product with silica hydrogel, drying and calcining the resulting composite at an elevated temperature.

#### References Cited by the Examiner

##### UNITED STATES PATENTS

|           |       |                        |         |
|-----------|-------|------------------------|---------|
| 2,698,305 | 12/54 | Plank et al. -----     | 252-455 |
| 2,728,710 | 12/55 | Hendricks -----        | 208-112 |
| 2,799,626 | 7/57  | Johnson et al. -----   | 208-110 |
| 2,882,221 | 4/59  | Dinwiddie et al. ----- | 208-111 |
| 2,911,356 | 11/59 | Hanson -----           | 208-110 |

##### OTHER REFERENCES

Advances in Catalysts, vol. VI (1954), page 384, Academic Press Inc., New York, publishers.

60 "Conversion of Petroleum," Sachanen, 2nd edition, page 314.

ALPHONSO D. SULLIVAN, Primary Examiner.

ALLAN M. BOETTCHER, MILTON STERMAN,  
65 Examiners.

UNITED STATES PATENT OFFICE  
CERTIFICATE OF CORRECTION

Patent No. 3,182,012

May 4, 1965

Lewis M. Browning et al.

It is hereby certified that error appears in the above numbered patent requiring correction and that the said Letters Patent should read as corrected below.

Column 4, line 6, for "commingling" read -- comingling --; line 36, for "hydogel" read -- hydrogel --; column 5, line 16, after "example" insert -- alumina --; line 24, for "sucessively" read -- successively --; column 8, line 58, for "sen from the above table" read -- seen from the above Table --; column 9, line 7, for "gases" read -- gas --.

Signed and sealed this 12th day of October 1965.

SEAL)

test:

ERNEST W. SWIDER  
Testing Officer

EDWARD J. BRENNER  
Commissioner of Patents